

# UNITED STATES PATENT OFFICE.

KANESUKE KIMURA, OF KOBE, JAPAN.

## PROCESS FOR PREPARING CATALYTIC AGENT FOR HYDROGENATING HARD OILS.

1,327,396.

Specification of Letters Patent.

Patented Jan. 6, 1920.

No Drawing.

Application filed August 1, 1917. Serial No. 183,982.

*To all whom it may concern:*

Be it known that I, KANESUKE KIMURA, a subject of the Emperor of Japan, residing at No. 2 Hakayama, Higashi - Shiri - Ike-  
5 Mura, Kobe, Japan, engineer, have invented certain new and useful Improvements in Processes for Preparing Catalytic Agent for Hydrogenating Hard Oils, of which the following is a specification.

10 The present invention relates to the hydrogenating of oils by the use of nickel as a catalyst.

The invention has for its object the manufacture in a simple and economical manner 15 of a catalytic agent which can be produced from any desired nickel salt and is of relatively high efficiency owing to the fact that it allows of the reduction process being performed at a relatively low temperature.

20 With this object in view the present invention consists in the preparation of a nickel catalytic agent, the invention being characterized by the fact that a nickel salt is mixed with an incombustible or inert and non-catalytic substance, such as powdered asbestos 25 or infusorial earth, and the mixture is heated while ammonia gas, gaseous ammonium chlorid, is passed through it.

In preparing a catalytic agent according 30 to the present invention, a nickel salt—such as nickel nitrate, nickel sulfate, nickel chlorid, nickel formate, nickel acetate, or nickel oxalate—is first reduced to very fine powder; and the powdered salt thus obtained is thoroughly mixed with an incombustible and 35 non-catalytic substance, such, for example, as powdered asbestos, diatomaceous or infusorial earth, or pumice. The mixture, after being dried, is passed into a vessel of 40 iron, nickel, glass, quartz, or other material which effects no catalytic action whatever, in which vessel it is heated while ammonia gas, gaseous ammonium chlorid, in gaseous form is passed through it. Pure ammonia 45 gas can be used with effect, but ammonium chlorid gas is to be preferred in view of the fact that it forms a colorless vapor at approximately 450 degrees C.

In the carrying of the present invention 50 into effect in one convenient manner, 493 parts of powdered nickel nitrate are thoroughly mixed with 100 parts of powdered pumice. The vessel in which the mixture is treated, and which is of a material as heretofore specified, is connected by a leading pipe with a generator of ammonium-chlorid vapor. The vessel is heated from out-

side to a suitable temperature by the use of a steam jacket or other suitable means, and an agitator, provided in the vessel, is caused 60 to rotate continuously while the vapor of ammonium chlorid is passed through the leading pipe into the vessel, with the result that the nickel salt is reduced to a powdered nickel ready for use, as a catalytic agent, in 65 the subsequent process for hardening fatty oils.

In this hardening process the powdered nickel, together with a fatty oil is passed into a machine which is provided with a 70 steam jacket or other suitable heating contrivance. This machine is provided with an agitator, which is rotated and causes the substances within the machine to be mixed together, while hydrogen gas is introduced 75 into the machine by means of a leading pipe. The agitator, which is provided with a net, made of a metal such as iron, copper, nickel, silver or platinum, is rotated rapidly, developing a centrifugal force which effects 80 the perfect commingling of the contents of the machine and thereby produces a saturated fatty oil.

The catalytic agent obtained by means of the vapor current of ammonia, ammonium 85 chlorid in accordance with my present invention can act at a relatively low temperature, and its use is therefore conducive to high efficiency. Moreover, any nickel salt may arbitrarily be chosen for use in my 90 process, which is not the case in processes heretofore in use. The utility of my invention will therefore be evident.

Having now particularly described and ascertained the nature of my said invention 95 and in what manner the same is to be performed, I declare that what I claim is:—

The process of preparing a nickel catalytic agent for hydrogenating oils, consisting in mixing powdered nickel nitrate with 100 powdered pumice, charging the mixture into a vessel of a material which effects no catalytic action with such mixture, heating said vessel and its contents by heating means applied exteriorly of said vessel, agitating the 105 contents of the vessel, and subjecting the contents of the vessel to the action of the vapor of ammonium chlorid.

In testimony whereof I affix my signature in presence of two witnesses.

KANESUKE KIMURA.

Witnesses:

W. EBiharAH,

A. Arase.